

## UNITED STATES PATENT OFFICE

2,045,074

## MERCERIZING LIQUORS

Jacques Feldmann, Basel, Switzerland, assignor  
to the firm of J. R. Geigy A. G., Basel, Switzerland

No Drawing. Application August 18, 1934, Serial  
No. 740,539. In Germany September 7, 1933

## 10 Claims. (Cl. 8—20)

It is known that difficulties arise in the treatment of textile materials of natural or regenerated cellulose with alkalis, for example, mercerization, owing to the difficulty with which the fibres are wetted, so that the action of the alkali proceeds only slowly and lacks uniformity. Many proposals have been made for overcoming this objection, either by pretreating the textile materials, for example, by Kier boiling, or by adding 5 to the alkaline bath a substance which imparts to it a greater capacity for wetting the material.

The use of phenols and homologues thereof for this purpose has long been known, and it has since frequently been attempted to increase the 15 insufficient action of these compounds by suitable additions, such as soaps, Turkey red oils, alcohols, amines, ethers and so on.

According to this invention the wetting and penetrative capacity of alkaline baths for the 20 treatment of textiles can be considerably increased by adding to the liquid cymene-sulphamide and a mono- or di-carboxylic acid of the terpene or camphor series, together with a solvent distributor. The quantity of the added substances may amount to 5-20 grams per liter of 25 liquor.

The addition of aromatic sulphonate and carboxylic acids to alkaline liquors, even together with a solvent distributor, has the disadvantage, 30 explicable by the law of mass action, that the salts of these acids which are formed are only sparingly soluble owing to the high concentration of the bath in alkali and are therefore in greater part precipitated. Cymene-sulphamide exhibits 35 specific properties in concentrated solutions of alkalis, and moreover, as a sulphamide it is far less dependent on the aforesaid influences which limit the solubility. It acts as an excellent solvent distributor for the alkali salts of the carboxylic acid of the terpene and camphor series.

A mercerizing liquor containing additions in accordance with the present invention has a 40 very high capacity for wetting and penetrating the textile material; the concentrated alkali solution takes effect very rapidly and uniformly and raw cotton which has not been de-sized can be used without any pre-treatment. This excellent wetting action, especially in the first 45 fifteen seconds, is possessed by neither of the classes of substances alone. These are indeed good wetting agents when added separately to a mercerizing liquor together with a solvent distributor, but the terpene and camphor carboxylic acids particularly have a tendency to precipitate,

so that the wetting action is greatly reduced. Only by the combination of substances of the two chemical classes is it possible to attain the remarkable wetting action together with the other favourable properties nowadays required of a 5 wetting agent for use in mercerizing baths.

The wetting action may be somewhat further increased, without detracting from the general properties, by the addition of a small proportion of a hydrocarbon of the benzene series particularly cymene.

As solvent distributor there may be used, for example, phenol, a cresol, a xylol, a mixture of cresols, methyl alcohol, ethyl alcohol, a highly 15 sulphonated oil or the like.

Among the carboxylic acids of the terpene and camphor series suitable for use in the invention there may be named in particular bornylene carboxylic acid, campholic acid, isocampholic acid, 20 fencholic acid, oxyfencholic acid, hydropinenic acid, sabinenic acid, camphoric acid, cineolic acid and so on.

The following examples illustrate the invention, but it will be understood that the proportions given therein may vary within wide limits:— 25

## Example 1

To a caustic soda solution of 30° Bé. are added 30 per liter 15 grams of a mixture consisting of:

|                   | Per cent |
|-------------------|----------|
| Fencholic acid    | 5        |
| Cymene-sulphamide | 10       |
| Crude cresol      | 85       |

The mercerizing liquor thus prepared wets raw cotton uniformly within a few seconds, so that the mercerizing operation may be conducted with 40 great certainty and without the faulty results which would otherwise frequently occur.

## Example 2

Instead of the mixture used in Example 1 there is used a mixture of:

|                           | Per cent |
|---------------------------|----------|
| Bornylene carboxylic acid | 5        |
| Cymene sulphamide         | 10       |
| Crude cresol              | 75       |
| Ethyl alcohol             | 10       |

There is obtained the same result as in Example 1.

*Example 3*

Instead of the mixture given in Example 1 there is added a mixture of:

|                     | Per cent |
|---------------------|----------|
| 5 Dl-campholic acid | 4.8      |
| Cymene sulphamide   | 10       |
| Cymene              | 0.52     |
| Crude cresol        | 74.68    |
| Ethyl alcohol       | 10       |

10 There is obtained the same result as in Example 1.

*Example 4*

15 To a caustic soda solution of 30° Bé. are added per liter 15 grams of a mixture consisting of:

|                   | Per cent |
|-------------------|----------|
| Cinellic acid     | 4.5      |
| Cymene-sulphamide | 9.5      |
| 20 Crude cresol   | 85.0     |

There is obtained the same result as in Example 1.

*Example 5*

25 Instead of the mixture used in Example 1 there is used a mixture of:

|                   | Per cent |
|-------------------|----------|
| Camphoric acid    | 5        |
| Cymene-sulphamide | 10       |
| 30 Crude cresol   | 75       |
| Ethyl alcohol     | 10       |

There is obtained the same result as in Example 1.

*Example 6*

35 Instead of the mixture given in Example 1 there is added a mixture of:

|                    | Per cent |
|--------------------|----------|
| 40 Terpenylic acid | 5        |
| Cymene-sulphamide  | 10       |
| Crude cresol       | 85       |

There is obtained the same result as in Example 1.

45 What I claim is:—

1. A process for increasing the wetting and penetrative capacity of alkaline mercerizing liquids, which consists in adding to the mercerizing liquid a cymene sulphamide, a carboxylic acid of the terpene series and a solution promoter and distributor.

2. A process for increasing the wetting and penetrative capacity of alkaline mercerizing liquids, which consists in adding to the mercerizing liquid a cymene sulphamide, a monocarboxylic acid of the terpene series and a solution promoter and distributor.

3. A process for increasing the wetting and penetrative capacity of alkaline mercerizing liquids, which consists in adding to the mercerizing liquid a cymene sulphamide, a monocarboxylic acid of the terpene series and a phenolic body as solution promoter and distributor.

4. A process for increasing the wetting and penetrative capacity of alkaline mercerizing liquids, which consists in adding to the mercerizing liquid a cymene sulphamide, a monocarboxylic acid of the terpene series and an alcohol of low molecular weight as solution promoter and distributor.

5. A process for increasing the wetting and penetrative capacity of alkaline mercerizing liquids, which consists in adding to the mercerizing liquid a cymene sulphamide, a monocarboxylic acid of the terpene series and a highly sulphonated oil as solution promoter and distributor.

6. A preparation suitable for addition to an alkaline mercerizing liquid, comprising cymene sulphamide, a carboxylic acid of the terpene series and a solution promoter and distributor, jointly.

7. A preparation suitable for addition to an alkaline mercerizing liquid, comprising cymene sulphamide, a monocarboxylic acid of the terpene series and a solution promoter and distributor, jointly.

8. A preparation suitable for addition to an alkaline mercerizing liquid, comprising cymene sulphamide, a monocarboxylic acid of the terpene series and a solution promoter and distributor of the phenolic type, jointly.

9. A preparation suitable for addition to an alkaline mercerizing liquid, comprising cymene sulphamide, a monocarboxylic acid of the terpene series and a solution promoter and distributor, consisting of an alcohol of low molecular weight.

10. A preparation suitable for addition to an alkaline mercerizing liquid, comprising cymene sulphamide, a monocarboxylic acid of the terpene series and a solution promoter and distributor, consisting of a highly sulphonated oil.

JACQUES FELDMANN.